

1

3,275,717

**STABILIZER FOR TRIMETHYLPHOSPHATE**  
Harry S. Butler, Baton Rouge, La., assignor to Ethyl Corporation, New York, N.Y., a corporation of Virginia  
No Drawing. Filed Apr. 29, 1963, Ser. No. 276,183  
6 Claims. (Cl. 260—963)

This invention relates to the stabilization of automotive ignition control compound mixes and in particular is directed to those mixes containing trimethylphosphate, either in its pure form or in concentrated solution with other additives.

Trimethylphosphate as commercially supplied today normally contains a very small trace of water. However, this minute trace of water hydrolyzes the trimethylphosphate over a period of time to produce the corresponding orthophosphoric acids. This acid produces a cloudiness or white precipitate in the trimethylphosphate when it is allowed to stand in contact with steel. While this white precipitate in no manner subtracts from the ability of the remaining trimethylphosphate to function as an ignition control agent, it does present a material handling problem in that if it is allowed to build up appreciably, it might clog screens or other handling equipment, besides being objectionable from an aesthetic viewpoint. Moreover, it corrodes such equipment which in itself is objectionable. Thus, a method of inhibiting trimethylphosphate containing minute quantities of corrosive acids without impairing its effectiveness as an ignition control agent would represent a desirable contribution to the art.

An object of this invention is to stabilize trimethylphosphate as commercially supplied and when in contact with a ferrous material. A more specific object is to stabilize trimethylphosphate containing minute traces of acids by adding thereto a compound which does not impair its effectiveness as an ignition control agent.

These objectives are accomplished pursuant to this invention by adding an amine compound to trimethylphosphate, or a highly concentrated solution thereof, containing slight traces of water and/or acids. The most suitable amines are the lower alkyl amines, that is, those containing from 1 through 6 carbon atoms per alkyl group. Especially preferred are the tertiary alkyl amines wherein the alkyl groups are similar (and most preferably, the same) since these compounds are more readily available. Of these, the tributyl amines are especially preferred since they have a boiling point close to that of trimethylphosphate. Thus, a preferred embodiment of this invention is trimethylphosphate and concentrated mixtures thereof containing an amine having a boiling point close to that of the trimethylphosphate. While amines having a boiling point lower than that of trimethylphosphate are perfectly suitable for use pursuant to the practice of this invention, they naturally have more tendency to vaporize out of solution and hence be lost for their intended use. On the other hand, amines having a boiling point higher than that of trimethylphosphate, while usually more effective, are generally less soluble and hence present a mixing problem. Moreover, their increased cost also makes them less attractive. While tertiary amines are preferred, secondary and primary amines under the right conditions can be employed pursuant to the practice of this inven-

2

tion. However, they are generally less stable and hence offer no technical advantage over the preferred tertiary amines.

Exemplary of the compounds that can be employed as stabilizers pursuant to this invention are: trimethylamine, triethylamine, tri-n-propylamine, triisopropylamine, tri-n-butylamine, tri-sec-butylamine, tri-tert-butylamine, triisobutylamine, tri-n-amylamine, tri-n-hexylamine, tri-n-octylamine, tri-n-decylamine, ethyl dibutylamine, and the like.

Surprisingly, the concentration of the amine to achieve these desirable end results is generally less than that quantity necessary to completely neutralize any contained acids in the trimethylphosphate. Without wishing to be bound by theory, it is thought that the amine coats the ferrous material in contact with the trimethylphosphate and consequently, theoretical neutralization of the objectionable phosphoric acid is not required. Generally speaking, it has been found that a concentration as low as 0.2 weight percent amine based on the total solution up to about 2.0 weight percent, usually not above 1.0 weight percent, is suitable to adequately inhibit both neat trimethylphosphate and highly concentrated solutions as commercially available today. By highly concentrated solutions is meant solutions in which trimethylphosphate is present at about 50 percent by weight in a suitable solvent, such as hydrocarbon solvents or in other antiknock fluid compositions.

It is to be understood of course that concentrations greater than 2.0 weight percent based on the weight of trimethylphosphate can be employed. However, concentrations less than this value are preferred since generally speaking such amounts, besides achieving the objectives of this invention, are readily soluble in trimethylphosphate at ambient temperature conditions. The extent of contact between the trimethylphosphate and a ferrous material primarily influences the necessary amount of amine that must be present in order to stabilize the trimethylphosphate. The only time the concentration of acids in the trimethylphosphate appears to influence such determination is where the trimethylphosphate is stored for unduly long periods of time, say on the order of six months. Even so, for the latter situation seldom is more than 2.0 weight percent required.

Another distinct advantage of the instant invention is that no insoluble products are formed by the addition of the amine to the trimethylphosphate. This is highly unexpected in light of the fact that one might expect that the amine, being a base, when added to the trimethylphosphate containing acids would result in the formation of salt like materials which would precipitate out of solution and thus compound the problem solved by this invention rather than rectify it. For example, employing a commercially available source of neat trimethylphosphate containing 0.26 weight percent water and 0.016 meq./g. acid, the addition of 0.5 weight percent of the preferred tri-n-butylamine is highly effective in preventing the formation of any precipitate when the trimethylphosphate is allowed to stand in contact with ferrous material or in a steel container. When the resultant solution is added to a fuel, either as such or first blended with antiknock fluid compounds, test results confirm the fact that the trimethylphosphate is identically effective to that of trimethylphos-

phate which has not been stabilized as taught by way of this invention.

The following examples wherein all parts are by weight unless otherwise specified demonstrate the effectiveness of an amine for stabilizing trimethylphosphate.

The following tests were conducted with neat trimethylphosphate to which was added approximately 4 times the specification level of mixed acids normally present in commercial grade trimethylphosphate. The test mixture was analyzed and found to contain 0.28 weight percent water and 0.137 meq./g. acid. The neat trimethylphosphate was then tested at several temperature levels.

The first temperature level was at room temperature which was approximately 70 to 75° F. About 50 milliliters of the neat trimethylphosphate solution containing the excess acid was added to each of numerous containers wherein a mild steel specimen was placed. The containers were then capped to prevent contact with the atmosphere. They were then observed at least twice a week for cloudiness or the formation of a white precipitate.

The second temperature level investigated was at about 110° F. About 25 milliliters of the neat trimethylphosphate containing the excess acid was added to numerous test tubes each containing a mild steel specimen. The test tubes were then closed to the atmosphere and placed in a constant temperature bath controlled at 110° F. The solutions were then observed at least twice a week for the formation of a white precipitate or cloudiness.

The results of these test runs are tabulated below.

TABLE I

| Test No. | Acid Present (meq./g.) | Temp. (°F.) | Inhibitor Added, Wgt. Percent | Observations      |
|----------|------------------------|-------------|-------------------------------|-------------------|
| 1        | 0.016                  | 70-75       | None                          | Cloudy (3 days).  |
| 2        |                        |             | 0.1 Am <sub>3</sub> N*        | Cloudy (17 days). |
| 3        |                        |             | 0.5 Am <sub>3</sub> N         | Clear (137 days). |
| 4        |                        |             | 1.0 Am <sub>3</sub> N         | Clear (137 days). |
| 5        |                        |             | 0.1 Bu <sub>3</sub> N         | Cloudy (17 days). |
| 6        |                        |             | 0.5 Bu <sub>4</sub> N**       | Clear (64 days).  |
| 7        |                        | 110         | 0.5 Bu <sub>3</sub> N         | Clear (78 days).  |
| 8        |                        | 70-75       | 1.0 Bu <sub>3</sub> N         | Clear (137 days). |
| 9        |                        | 110         | 1.0 Bu <sub>3</sub> N         | Clear (94 days).  |
| 10       |                        | 110         | 2.0 Bu <sub>3</sub> N         | Clear (94 days).  |
| 11       |                        | 70-75       | 0.1 Et <sub>3</sub> N***      | Cloudy (15 days). |
| 12       |                        |             | 0.5 Et <sub>3</sub> N         | Clear (137 days). |
| 13       |                        |             | 1.0 Et <sub>3</sub> N         | Clear (137 days). |
| 14       | 0.14                   |             | None                          | Cloudy (1 day).   |
| 15       |                        |             | 0.1 Am <sub>3</sub> N         | Cloudy (2 days).  |
| 16       |                        |             | 0.5 Am <sub>3</sub> N         | Cloudy (92 days). |
| 17       |                        |             | 1.0 Am <sub>3</sub> N         | Clear (136 days). |
| 18       |                        |             | 0.1 Bu <sub>3</sub> N         | Cloudy (2 days).  |
| 19       | 0.14                   | 70-75       | 0.5 Bu <sub>3</sub> N         | Clear (63 days).  |
| 20       |                        | 110         | 0.5 Bu <sub>3</sub> N         | Clear (73 days).  |
| 21       |                        | 70-75       | 1.0 Bu <sub>3</sub> N         | Clear (136 days). |
| 22       |                        | 110         | 1.0 Bu <sub>3</sub> N         | Clear (94 days).  |
| 23       |                        | 110         | 2.0 Bu <sub>3</sub> N         | Clear (94 days).  |
| 24       |                        | 70-75       | 0.1 Et <sub>3</sub> N         | Cloudy (2 days).  |
| 25       |                        |             | 0.5 Et <sub>3</sub> N         | Clear (136 days). |
| 26       |                        |             | 1.0 Et <sub>3</sub> N         | Clear (136 days). |

\*Tri-n-aminylamine.

\*\*Tri-n-butylamine.

\*\*\*Triethylamine.

A next series of tests were run wherein the trimethylphosphate contained a similar amount of excess acid as in the above runs except that the trimethylphosphate was dissolved in about a 50 weight percent hydrocarbon solvent. The results are given in Table II.

TABLE II

| Test No. | Acid Present (meq./g.) | Temp. (°F.) | Inhibitor Added, Wgt. Percent | Observations     |
|----------|------------------------|-------------|-------------------------------|------------------|
| 5        |                        |             |                               |                  |
| 27       | 0.02                   | 70-75       | None                          | Cloudy (1 day).  |
| 28       |                        |             | 1.0 Bu <sub>3</sub> N         | Clear (94 days). |
| 29       |                        |             | 2.0 Bu <sub>3</sub> N         | Clear (94 days). |
| 30       | 0.14                   |             | None                          | Cloudy (1 day).  |
| 31       |                        |             | 1.0 Bu <sub>3</sub> N         | Clear (94 days). |
| 32       |                        |             | 2.0 Bu <sub>3</sub> N         | Clear (94 days). |
| 33       | 0.02                   | 110         | None                          | Cloudy (1 day).  |
| 34       |                        |             | 1.0 Bu <sub>3</sub> N         | Clear (94 days). |
| 35       |                        |             | 2.0 Bu <sub>3</sub> N         | Clear (94 days). |
| 36       | 0.14                   |             | None                          | Cloudy (1 day).  |
| 37       |                        |             | 1.0 Bu <sub>3</sub> N         | Clear (94 days). |
| 38       |                        |             | 2.0 Bu <sub>3</sub> N         | Clear (94 days). |

The above tests clearly demonstrate the effectiveness of an amine as a stabilizer for trimethylphosphate containing traces of water and/or acid when in contact with a ferrous material.

20 When employing trimethylphosphate containing a concentration of amine as taught herein as an ignition control agent, no reduction in its effectiveness as such is indicated.

I claim:

25 1. A mixture comprising trimethylphosphate present in the form of at least a concentrated solution thereof and further comprising minute quantities of water sufficient to form phosphoric acids, containing an amount of a tertiary alkyl amine less than the theoretical amount which would be necessary to neutralize said acids.

2. A mixture comprising trimethylphosphate present in the form of at least a concentrated solution thereof and further comprising a trace of water or acid stabilized by the addition of a tertiary alkyl amine wherein each 35 alkyl group contains from 1 to 6 carbon atoms, said amine being present in less than the theoretical amount which would be necessary to neutralize said acids.

3. Stabilization of a mixture comprising trimethylphosphate present in the form of at least a concentrated solution thereof by the addition thereto of a tertiary alkyl amine having a boiling point of about 379° F., said amine being present in less than the theoretical amount which would be necessary to neutralize any acids present.

4. Stabilization of a mixture comprising trimethylphosphate present in the form of at least a concentrated solution thereof by the addition thereto of tri-n-butylamine, said amine being present in less than the theoretical amount which would be necessary to neutralize any acids present.

50 5. Stabilized neat trimethylphosphate containing 0.2 to 1.0 weight percent tri-n-butylamine, said amine being present in less than the theoretical amount which would be necessary to neutralize any acids present.

6. Stabilized neat trimethylphosphate containing 0.5 weight percent tri-n-butylamine, said amine being present in less than the theoretical amount which would be necessary to neutralize any acids present.

#### References Cited by the Examiner

#### UNITED STATES PATENTS

2,114,866 4/1938 Vaughn ----- 260—461,316

CHARLES B. PARKER, Primary Examiner.

65 FRANK M. SIKORA, Assistant Examiner.

UNITED STATES PATENT OFFICE  
CERTIFICATE OF CORRECTION

Patent No. 3,275,717

September 27, 1966

Harry S. Butler

It is hereby certified that error appears in the above numbered patent requiring correction and that the said Letters Patent should read as corrected below.

Column 4, line 33, for "or acid stabilized" read -- or phosphoric acids or mixtures thereof stabilized --.

Signed and sealed this 26th day of September 1967.

(SEAL)

Attest:

ERNEST W. SWIDER

Attesting Officer

EDWARD J. BRENNER

Commissioner of Patents